

# UNITED STATES PATENT OFFICE.

GRENVILLE MELLEN, OF EAST ORANGE, NEW JERSEY, ASSIGNOR OF ONE-HALF TO  
UNITED ALUMINUM INGOT COMPANY, A CORPORATION OF NEW YORK.

## PROCESS FOR PURIFYING ALUMINUM AND ITS ALLOYS.

1,092,936.

Specification of Letters Patent. Patented Apr. 14, 1914.

No Drawing. Original application filed June 26, 1912, Serial No. 706,041. Divided and this application filed October 10, 1912. Serial No. 725,059.

To all whom it may concern:

Be it known that I, GRENVILLE MELLEN, a citizen of the United States, residing at East Orange, in the county of Essex and State of New Jersey, have invented certain new and useful Improvements in Processes for Purifying Aluminum and Its Alloys, of which the following is a specification.

This invention relates to a process for purifying molten aluminum or its alloys from impurities, such as aluminum oxide, and is a division of my application Serial Number 706,041, filed June 26, 1912. The impurities are largely aluminum oxide, resulting from the superficial oxidation of the metal when molten; said oxids being stirred in the mass of the metal and mechanically held therein.

If a material which is non-oxidizing, and which boils at a temperature lower than the melting-point of aluminum, and of lower specific gravity than aluminum, be injected into the lower level of the molten metal, the vapors on arising through the metal will have the result of carrying the impurities to the surface where they may dissolve or combine with a flux on the surface; or if such impurities chemically or mechanically combine with the vaporizable material added, the resulting compound or mixture will rise to the surface, from which it may be removed in any suitable manner. I have found that the addition of sulfur to molten aluminum or its alloys has this property; and on injecting solid sulfur to the bottom of a container filled with the molten metal or alloy, the sulfur boils, and its vapors passing through the molten metal stir it vigorously, combining with the impurities either mechanically or chemically and carry them to the surface, from which they may be removed. It is advantageous to also add a fusible material having a low specific gravity which acts as a flux and serves to mechanically entrain or to chemically combine with the impurities, carrying them to the surface, from which they may be removed. I have further found that by adding sodium chlorid (salt) to molten sulfur, thoroughly stirring, and casting into rods, I obtain a material particularly adapted to remove the impurities above referred to. A rod of this material is plunged into the molten metal or alloy, and stirred, the salt melting and the

sulfur boiling from the surface of the rod, 55 the sulfur vapors bubbling through the molten metal, while the molten salt passes up more slowly. The combined action of the sulfur vapors and salt is to free the metal from its impurities by carrying them to the 60 surface, where they form a flux or scoria with the salt, or with any other flux present, and from which they can readily be removed. The treatment of the molten metal or alloy is of greater or less duration depending 65 upon the quantity of impurities present. The rod of salt and sulfur may contain from 30 to 70 per cent. of salt, an excess of salt or sulfur in the rod not materially affecting the results; an excess of salt, however, increases the life of the rod when immersed in the molten metal. When the rod of salt and sulfur is inserted, the sulfur gradually boils away; its vapors causing violent ebullition 70 of the mass of metal, thoroughly agitating it, 75 and carrying its impurities to the surface.

Instead of sodium chlorid, I may melt together sulfur and sodium sulfid.

To the surface of the molten metal may be added a flux such as sodium meta-phosphate 80 or zinc chlorid which fuses readily and combines with the salt and sulfur scoria or dross; it will further serve to effect a ready separation of the scoria from the molten metal.

I have found that aluminum scrap from different sources, such as scrap sheet, turnings, and castings that have been corroded by use and exposure to air and water, and which, if melted without any purifying 90 agent, would produce a very impure metal, will, upon being treated with the purifying agency herein described, produce a metal equal in every way to new and hitherto unused metal.

I claim:

1. The process of purifying aluminum and its alloys, comprising adding to the molten metal a flux comprising a substance vaporizable at the temperature of melted aluminum, and a substance fluid at the temperature at which aluminum is cast, and agitating the metal by the vapors of the vaporizable substance.
2. The process of purifying aluminum and its alloys, comprising adding sulfur to the molten metal.
3. The process of purifying aluminum

and its alloys, comprising subjecting the melted metal to the action of sulfur vapors bubbling therethrough.

4. The process of purifying aluminum and its alloys, comprising adding sulfur and a fusible solid to the molten metal, said solid having a lower specific gravity than the metal.

5. The process of purifying aluminum and its alloys, comprising subjecting the

melted metal to a sulfur-containing purifying agent, and reacting upon the impurities in the melted metal with the sulfur in the sulfur-containing agent.

In testimony whereof I affix my signature 15 in presence of two witnesses.

GRENVILLE MELLEN.

Witnesses:

JOHN O. BIGELOW,  
STUART A. YOUNG.